

## 1

3,438,821

ARTICLE AND METHOD OF HEAT TREATING  
HIGH PHOSPHORUS STEELS

John Y. Riedel, Bethlehem, Pa., assignor to Bethlehem Steel Corporation, a corporation of Delaware  
No Drawing. Continuation of application Ser. No. 497,550, Oct. 18, 1965. This application May 17, 1968, Ser. No. 731,680  
Int. Cl. C21d 1/22

U.S. Cl. 148—134

7 Claims

## ABSTRACT OF THE DISCLOSURE

A method of tempering martensitically hardened high phosphorus-carbon steel to provide a combination of corrosion resistance, high strength and low impact transition temperature. The tempering treatment comprises heating the martensitically hardened steel to a temperature between the  $Ac_1$  temperature and about 150° F. below the  $Ac_1$  and cooling from such temperature at a rate not less than 1° F. per second.

This application is a continuation of application Ser. No. 497,550, filed Oct. 18, 1965, now abandoned.

This invention relates to a method of heat treating steel and more particularly to a method of improving the notch toughness of martensitically hardened high phosphorous steels.

In the past, the use of significant amounts of phosphorous as an alloying element has been limited to low carbon ferritic steel. The principal reason for this limitation appears to be the embrittling effect of phosphorous. It is well known that this effect is particularly severe in steels containing sufficient carbon to respond to a quench and temper type of heat treatment. As a result there are no commercial steels containing significant amounts of phosphorous to improve the hardenability and corrosion resistance of martensitically hardened steels.

The principal object of this invention is to provide a method of heat treatment which will extend the use of phosphorous as an alloying element to steels containing sufficient carbon to result in the formation of martensite when quenched from above the upper critical temperature.

Another object of this invention is to provide a method

of heat treating high carbon-high phosphorous steels to improve their notch toughness.

Another object is to provide a method of lowering impact transition temperatures and to enhance the hardenability and corrosion resistance of martensitically hardened high carbon-high phosphorous steels.

Still another object of this invention is to provide an inexpensive corrosion resistant material having sufficient tensile and impact strength to permit its use as a high strength material.

These and other objects are accomplished in the present invention by means of a method of heat treating carbon-phosphorous steels utilizing conventional marten-

## 2

sitic hardening techniques in which the tempering step involves cooling at a rapid rate from a narrow range of temperatures just below the  $Ac_1$ . It has been discovered that accelerated cooling from the tempering temperature has a very pronounced and unexpected effect on the impact transition temperature of martensitically hardened medium carbon-high phosphorous steels which does not occur in medium carbon-low phosphorous steels heat treated in a similar manner. This discovery has made it possible to extend the use of phosphorous as an alloying element into the field of martensitically hardened steels which have been hitherto considered to be too brittle.

Broadly, the tempering treatment of this invention comprises heating martensitically hardened, high phosphorous steel to a temperature between the  $Ac_1$  temperature and about 150° F. below the  $Ac_1$  and cooling from the tempering temperature at a rate of not less than 1° F. per second. With alloy steels having about .30% to .45% carbon, the tempering temperature should preferably be between 1250° F. and 1300° F. and oil quenching from the temper provides a satisfactory cooling rate for sections up to 2" in diameter.

The tempering treatment of my invention is applicable to steels containing not less than .12% carbon and not less than .06% phosphorous. It is particularly useful in the treatment of high strength, low alloy corrosion resistant steels containing from .35% to .55% carbon, .06% to .12% phosphorous, and other elements such as copper, nickel and/or chromium added to enhance the corrosion resistance of the steels. Compositions illustrating the broad and narrow limits of these steels are as follows:

|             | Narrow    | Broad     |
|-------------|-----------|-----------|
| 35 Carbon   | .35/.55   | .12/.80   |
| Manganese   | .50/1.50  | 1.50 max. |
| Phosphorous | .06/.12   | .06/.20   |
| Sulphur     | .05 max.  | .05 max.  |
| Silicon     | .20/.90   | .20/.90   |
| Nickel      | 1.00 max. | 1.00 max. |
| Chromium    | .40/1.00  | 1.00 max. |
| 40 Copper   | .50 max.  | .50 max.  |

Table I shows the compositions of two heats of medium carbon steel, the low phosphorous steel being illustrative of the prior art and the high phosphorous steel being an example of a steel which is benefited by the heat treatment of this invention.

TABLE I

|                  | C   | Mn   | P    | S    | Si  | Ni  | Cr  | V   | Mo  | Cu  |
|------------------|-----|------|------|------|-----|-----|-----|-----|-----|-----|
| High Phosphorous | .41 | 1.29 | .007 | .018 | .49 | .05 | .08 | .01 | .01 | .03 |
| Low Phosphorous  | .42 | 1.25 | .006 | .019 | .46 | .06 | .06 | .01 | .01 | .01 |

These two induction furnace heats were cast into hot-topped, 6½" square x 150 lbs. ingots. The ingots were heated to 2200° F. and rolled to 3" square billets. The billets were reheated to 2200° F. and rolled to 1" diameter round bars. The 1" bars were rough machined to 1/16" oversize charpy specimens. All specimens were heated to 1525° F., held at heat for one hour, and quenched in water. Specimens from each heat were tempered at 1000° F., 1100° F., 1200° F. and 1300° F. and quenched in water. The specimens were then finish machined to V-notch charpy impact specimens and broken at various temperatures to obtain the 15 ft./lb. transition temperatures shown in Table II.

TABLE II

[15 Ft. Lb. V-Notch Charpy Transition Temperatures]

| Temper                 | High Phosphorous, ° F. | Low Phosphorous, ° F. |
|------------------------|------------------------|-----------------------|
| 1,000° F. water quench | +75                    | -270                  |
| 1,100° F. water quench | +15                    | -215                  |
| 1,200° F. water quench | -75                    | -260                  |
| 1,300° F. water quench | -175                   | -240                  |

These results show that water quenching from a tempering temperature of 1200° F. or higher has a pronounced effect in improving the impact strength transition temperatures of martensitically hardened high phosphorus steels but that the same treatment had no significant effect on low phosphorus steels.

The effect of various cooling rates from a 1200° F. temper on the impact strength transition temperatures of martensitically hardened high phosphorus and low phosphorus steels is shown in Table III:

TABLE III

| Method of Cooling from 1,200° F. Temper | Approximate cooling Rate, ° F./sec. for $\frac{3}{4}$ " dia. | 15 Ft. Lb. V-Notch Charpy Transition Temperatures |                      |
|-----------------------------------------|--------------------------------------------------------------|---------------------------------------------------|----------------------|
|                                         |                                                              | High Phosphorus, ° F.                             | Low Phosphorus, ° F. |
| Water Quench.....                       | 100                                                          | -75                                               | -260                 |
| Oil Quench.....                         | 40                                                           | -30                                               | -200                 |
| Air Blast.....                          | 3                                                            | +5                                                | -180                 |
| Still Air Cool.....                     | 0.7                                                          | +25                                               | -195                 |
| Furnace Cool (50° F./hr.).....          | 0.014                                                        | +200                                              | -200                 |

These results show that the effectiveness of accelerated cooling from the tempering temperature on the transition temperatures of martensitically hardened, high phosphorus steels is directly proportional to the cooling rate but that identical heat treatments fail to have any significant effect on low phosphorus steels.

Examples of specific compositions of high strength, corrosion resistant steels that were heat treated in the manner of this invention are shown in Table IV below:

TABLE IV

|          | Compositions |      |     |      |     |     |     |     |
|----------|--------------|------|-----|------|-----|-----|-----|-----|
|          | C            | Mn   | P   | S    | Si  | Ni  | Cr  | Cu  |
| Example: |              |      |     |      |     |     |     |     |
| A.....   | .38          | 1.05 | .10 | .039 | .47 | .74 | .80 | .36 |
| B.....   | .40          | .74  | .10 | .032 | .29 | .75 | .67 | .39 |
| C.....   | .46          | .85  | .10 | .032 | .35 | .76 | .74 | .39 |
| D.....   | .52          | .72  | .10 | .038 | .38 | .79 | .77 | .42 |

Steels of the compositions set forth in Table IV were heat treated in the manner set forth in Table V below:

TABLE V.—HEAT TREATMENTS

| Number: | Harden                      | Temper                      |
|---------|-----------------------------|-----------------------------|
| 1.....  | 1,550° F. Oil Quench.....   | 1,250° F. Water Quench..... |
| 2.....  | do.....                     | 1,275° F. Water Quench..... |
| 3.....  | do.....                     | 1,300° F. Water Quench..... |
| 4.....  | 1,550° F. Water Quench..... | 1,250° F. Water Quench..... |
| 5.....  | do.....                     | 1,275° F. Water Quench..... |
| 6.....  | do.....                     | 1,330° F. Water Quench..... |

Test specimens cut from 1 $\frac{1}{4}$ " diameter bars of steels

having the compositions shown in Table IV and heat treated in the manner shown in Table V were subsequently tested. The results of these tests are shown in Table VI below:

TABLE VI.—PHYSICAL PROPERTIES

| Composition                     | Treatment | Yield Strength, p.s.i. | Tensile Strength, p.s.i. | Elong. | Reduction of Area | 15 Ft. Lb. V-Notch Charpy Transition Temperature, ° F. |
|---------------------------------|-----------|------------------------|--------------------------|--------|-------------------|--------------------------------------------------------|
| ASTM Specification A325-64..... | 1         | 177,000                | 1105,000                 | 14.0   | 135.0             | .....                                                  |
| A.....                          | 1         | 94,700                 | 120,000                  | 22.8   | 61.0              | -10                                                    |
| A.....                          | 2         | 92,700                 | 119,000                  | 23.0   | 59.4              | -35                                                    |
| A.....                          | 3         | 86,400                 | 113,800                  | 24.8   | 62.8              | -125                                                   |
| B.....                          | 1         | 91,500                 | 116,300                  | 23.5   | 64.0              | -40                                                    |
| B.....                          | 2         | 95,100                 | 121,200                  | 21.8   | 56.8              | -55                                                    |
| B.....                          | 3         | 84,800                 | 112,400                  | 23.5   | 57.2              | -70                                                    |
| C.....                          | 1         | 100,500                | 124,900                  | 20.3   | 50.6              | -15                                                    |
| C.....                          | 2         | 99,200                 | 127,500                  | 20.0   | 51.0              | -35                                                    |
| C.....                          | 3         | 93,200                 | 120,600                  | 20.5   | 47.3              | -100                                                   |
| D.....                          | 1         | 109,800                | 133,000                  | 20.0   | 52.4              | -10                                                    |
| D.....                          | 3         | 102,500                | 126,800                  | 21.3   | 52.7              | -35                                                    |
| B.....                          | 4         | 108,100                | 127,100                  | 19.5   | 51.6              | -15                                                    |
| B.....                          | 5         | 99,200                 | 120,700                  | 21.0   | 56.6              | -55                                                    |
| B.....                          | 6         | 88,700                 | 117,200                  | 22.5   | 54.9              | -100                                                   |
| C.....                          | 4         | 110,700                | 132,400                  | 21.0   | 56.4              | +5                                                     |
| C.....                          | 5         | 103,500                | 124,200                  | 16.0   | 37.9              | -35                                                    |
| C.....                          | 6         | 88,900                 | 122,500                  | 19.0   | 44.1              | -75                                                    |

<sup>1</sup> Minimum.

These results show that the minimum tensile test requirements for bolting materials shown in A.S.T.M. Specification A325-64 can be satisfactorily obtained with the heat treatment of the invention on steels having the compositions shown in Table IV, and, in addition, desirably low transition temperatures will be obtained. Thus, these materials are particularly adapted for use in the fabrication of structures requiring high strength, low alloy, corrosion resistant steels which are to be left exposed to the weather.

The heat treatment process of this invention is applicable broadly to martensitically hardened high phosphorus steels which may also contain various other alloying elements such as manganese, silicon, nickel, chromium, molybdenum, copper, vanadium, etc., either singly or in various combinations and amounts which are known to improve hardenability.

All references in the specification and claims to percentages are weight percentages.

I claim:

1. A method of tempering martensitically hardened steel consisting essentially of: .12% to .80% carbon, .06% to .20% phosphorus, balance iron, to produce a high strength, corrosion resistant steel having a 15 ft. lb. V-notch Charpy impact transition temperature no higher than 5° F., said method comprising:

45 (a) heating said steel to a temperature between the  $Ac_1$  temperature and the  $Ac_1$  minus 150° F., and  
 (b) cooling the steel from said temperature at a rate not less than 1° F. per second.

50 2. The method of claim 1 in which said steel contains:

55 C ..... .35-.55  
 Mn ..... .50-1.50  
 P ..... .06-.12  
 S (max.) ..... .05  
 60 Si ..... .20-.90  
 Ni (max.) ..... 1.00  
 Cr ..... .40-1.00  
 Cu (max.) ..... .50  
 balance iron.

65 3. The method of claim 1 in which said steel contains:

Percent  
 Mn (max.) ..... 1.50  
 S (max.) ..... .05  
 Si ..... .20-.90  
 Ni (max.) ..... 1.00  
 Cr (max.) ..... 1.00  
 Cu (max.) ..... .50  
 balance iron.

4. The method of tempering martensitically hardened steel consisting essentially of .12% to .80% carbon, .06% to .20% phosphorus, balance iron, to produce a high strength, corrosion resistant steel having a 15 ft. lb. V-notch Charpy impact transition temperature no higher than 5° F., said method comprising:

(a) heating said steel to a temperature between 1250° F. and 1300° F., and

(b) cooling said steel from said temperature at a rate not less than 1° F. per second.

5. The method according to claim 4 in which said steel contains:

|           | Percent |    |
|-----------|---------|----|
| Mn (max.) | 1.50    | 15 |
| S (max.)  | .05     |    |
| Si        | .20-.90 |    |
| Ni (max.) | 1.00    |    |
| Cr (max.) | 1.00    |    |
| Cu (max.) | .50     | 20 |

6. The method according to claim 4 in which said steel contains:

|           | Percent  |    |
|-----------|----------|----|
| C         | .35-.55  | 30 |
| Mn        | .50-.150 |    |
| P         | .06-.12  |    |
| S (max.)  | .05      |    |
| Si        | .20-.90  | 35 |
| Ni (max.) | 1.00     |    |
| Cr        | .40-.100 |    |
| Cu (max.) | .50      |    |

7. A high strength corrosion resistant, tempered martensitic steel consisting essentially of:

|           | Percent  |
|-----------|----------|
| C         | .12-.80  |
| P         | .06-.20  |
| Mn        | .50-.150 |
| S (max.)  | .05      |
| Si        | .20-.90  |
| Ni (max.) | 1.00     |
| Cr (max.) | 1.00     |
| Cu (max.) | .50      |

and the balance iron which has been heated to a temperature between the  $Ac_1$  temperature and a temperature 150° F. below the  $Ac_1$  temperature, and cooled from said temperature at a rate of not less than 1° F. per second, said steel characterized by a 15 ft. lb. V-notch charpy impact transition temperature no higher than 5° F.

#### References Cited

#### UNITED STATES PATENTS

|           |         |          |        |
|-----------|---------|----------|--------|
| 2,315,156 | 3/1943  | Larrabee | 75—123 |
| 2,319,635 | 5/1943  | Saylor   | 75—123 |
| 2,485,358 | 10/1949 | Case     | 75—123 |

#### OTHER REFERENCES

Allen et al.: Journal of the Iron and Steel Institute, vol. 182, April 1956, relied on pp. 375—388.

Hopkins et al.: Journal of the Iron and Steel Institute, vol. 188, March 1958, relied on pp. 218, 219 and 222—235. Transactions of AIME, vol. 188, February 1950, relied on pp. 389—396.

Transactions of AIME, vol. 185, August 1949, relied on pp. 535—543.

CHARLES N. LOVELL, Primary Examiner.

U.S. Cl. X.R.

148—143, 36